

# United States Patent Office.

E. C. MERRILL AND A. W. WILLARD, OF CHARLESTOWN, VERMONT,  
ASSIGNORS TO E. C. MERRILL.

*Letters Patent No. 95,824, dated October 12, 1869.*

## IMPROVED COMPOSITION FOR EMERY-WHEELS AND OTHER ABRADING-IMPLEMENT.

The Schedule referred to in these Letters Patent and making part of the same.

*To all whom it may concern:*

Be it known that we, E. C. MERRILL and A. W. WILLARD, both of Charlestown, in the county of Orleans, and State of Vermont, have invented an Improved Composition for Emery-Wheels and other Abrading-Tools; and we do hereby declare that the following is a description of our invention sufficient to enable those skilled in the art to practise it.

Our invention has reference to the manufacture of emery-wheels and other abrading-tools; and

The invention consists, primarily, in a grinding-wheel, or other tool, made of a mixture of emery, or other abrading-powder, and a sand or stone powder, of inferior hardness, artificially united by a suitable cementitious agent, the composition being moulded into suitable form.

The invention also consists in an emery or grinding-wheel as a new article of manufacture, made by artificially uniting the abrasive sand or powder by means of oxide of zinc and chloride of zinc, the wheel being formed in a suitable mould, into which the material in a plastic state is tamped.

In the practice of our invention, in making emery or grinding-wheels, we preferably employ both features of the improvement, proceeding as follows:

Supposing emery to be the main abrading-powder to be used, we take, for instance, twenty-five ounces of emery and five ounces of fine quartz or sand, and mix with the emery and sand about eight ounces of oxide of zinc.

Having incorporated these ingredients well together, we add seven or eight ounces of chloride of zinc, or enough to moisten well the whole mixture, with which mixture we then fill the mould, tamping the material well into it, so as to fill every part, and compact the whole well together.

We then leave the material in the mould, and in twenty-four hours it will have become hard and stone-like, and will be ready for use.

These proportions, and the method of procedure, may of course be varied, as circumstances may require.

By this process we obtain a very enduring wheel, and one which wears away very evenly and perfectly.

Our object in employing a material of inferior hardness, mixed with the main grinding-agent, is to keep the sharp edges of the harder material always prominent, and prevent the face of the stone from wearing smooth, as it always inclines to do where the grinding-powder is of uniform hardness, or the grains are united by a gum, or animal or vegetable cementitious agent.

In uniting abrasive powder to form a grinding-wheel or other abrading-tool, we have found that we can make a very enduring and comparatively cheap article, whether the grains be of uniform or of comparative hardness, by using abrasive powder, united by an oxide and a chloride of zinc, the united mass being compressed and formed in a suitable mould.

We claim an abrading-wheel, or tool made of emery, artificially united or combined with a softer abrading-powder, having sharp cutting points, substantially as described.

Also, as a new article of manufacture, a grinder-wheel or other tool, formed of abrasive powder, united by an oxide-of-zinc and a chloride-of-zinc solution, formed and compressed in a mould, substantially as described.

E. C. MERRILL.  
A. W. WILLARD.

Witnesses:

J. E. WILSON,  
B. F. D. CARPENTER.